

# UNITED STATES PATENT OFFICE.

JOHN H. MULLER, OF SECANE, PENNSYLVANIA.

## ELECTRIC CONTACT-POINT.

1,367,752.

Specification of Letters Patent.

Patented Feb. 8, 1921.

No Drawing.

Application filed December 23, 1918. Serial No. 268,055.

To all whom it may concern:

Be it known that I, JOHN H. MULLER, a citizen of the United States of America, and a resident of Secane, in the county of 5 Delaware and State of Pennsylvania, have invented a certain new and useful Improvement in Electric Contact-Points, of which the following is a true and exact description.

10 My invention relates to electric contact points or surfaces and is especially applicable to make and break circuits such as those used in magnetos, induction coils, etc. For severe service of this kind platinum has hitherto been the only material from which 15 such points have been made, which gives really good service, and even platinum points are found in service to require filing at times to restore the bright metallic surfaces on 20 which their most efficient action depends.

The object of my invention is to provide 25 metallic contact points of an alloy which will in efficiency and durability compare favorably with platinum, which will be less costly and which will maintain bright metallic surfaces even under conditions under 30 which platinum points become coated and require to be scraped or filed to restore full efficiency, and my invention consists in a contact point formed of an alloy of gold 35 and nickel in certain proportions and which I have discovered will produce such points having the highest efficiency in use and of remarkable durability and freedom from 40 liability of such coating as impairs the efficiency of such points.

The points with which I have obtained best results I form of an alloy containing approximately ninety per cent. gold and ten 45 per cent. nickel, and the closer these proportions are adhered to the better service the points will give in use. I have found that the nickel may be used in as low percentage as eight per cent. with a corresponding increase in gold without material impairment in the qualities of the points other than that they are somewhat softer and not quite so durable in use, but below eight per cent. nickel the alloy loses hardness rapidly, 50 and its lower melting point is also objectionable. Where the nickel is reduced to six per cent. the impairment of the alloy for my purposes is marked and points made from it will not give satisfactory results.

55 The effect of increasing the nickel percentage in the alloy above ten per cent. is not

markedly injurious on the points up to a percentage of about twelve per cent. This increase in nickel results in greater hardness in the alloy and in a slight loss in conductivity both to heat and electricity. Above twelve per cent. nickel content the alloy is distinctly inferior for my purposes and really satisfactory points cannot, I have found, be made from an alloy having a 60 nickel content of over fifteen per cent. The purer the gold and nickel used in compounding my alloy the better, but such impurities as are usually found in the commercial metals, particularly in the nickel, are not 65 markedly injurious, especially where a pure gold is used, as they form very small percentages in the alloy.

In my studies and experimentation on contact points of platinum and of alloys, 70 intended to take the place of platinum, I have found the following qualities to be of great importance: The metal used must be of high conductiveness both to heat and electricity. The metal must have both hardness 75 and toughness to withstand constant and rapid impact. The metal must be of such character as to retain a permanent bright metallic surface unaltered by heat or the vapors and gases to which it is exposed. The 80 metal must have a comparatively high melting point, though this quality is somewhat interdependent with its conductivity to heat. The composition of the alloy must be such as to permit the constant passage of a small 85 arc between the contact surfaces in the make and break action without it resulting either in the volatilization into the arc of sufficient material to wear away the surfaces or to prevent a sharp and complete 90 break of contact by undue conductiveness of the vaporized material in the arc. All the above specified qualities are possessed in a high degree by my points made for the described alloy of gold and nickel, and I believe them to be in many respects better than 95 platinum points, especially in producing efficient ignition at low speed.

It is, I have found, important that carbon should not be present in the alloy in 100 appreciable quantity, and care should be taken that this substance is not present in the nickel in more than a fractional percentage, and that it should not be introduced in greater quantity in the compounding of 105 the alloy. The percentage of copper, iron and cobalt ordinarily present in commercial

nickel are not materially harmful in the alloy owing to their great dilution, but as I have said, the purer the nickel used the better is the character of the alloy for my purpose.

Having now described my invention, what I claim as new and desire to secure by Letters Patent, is:

1. Electric contact points formed of an alloy of gold and nickel containing nickel

in proportion between fifteen per cent. and eight per cent. and gold in corresponding proportion.

2. Electric contact points formed of an alloy of gold and nickel with the gold forming approximately ninety per cent. of the alloy and the nickel approximately ten per cent.

JOHN H. MULLER.